

## UNITED STATES PATENT OFFICE

2,134,433

## LUBRICATING OIL

Troy Lee Cantrell and James Otho Turner, Lansdowne, Pa., assignors to Gulf Oil Corporation, Pittsburgh, Pa., a corporation of Pennsylvania

No Drawing. Application August 31, 1936,  
Serial No. 98,827

7 Claims. (Cl. 87—9)

This invention relates to improved lubricants and processes of making the same; and it comprises lubricating compositions and lubricants containing small amounts of improvement agents which mitigate or retard the normal destructive action of lubricating oil deterioration products on certain bearing surfaces, the improvement in this respect being noteworthy with even such bearing materials as alloys of cadmium with copper and silver, of cadmium with copper and nickel, of lead with copper and nickel, etc., even under relatively high temperatures, speeds and pressures, this improvement of the mineral oil being effected and its performance improved by the presence therein of a small amount of an alkyl thioether of ortho-amino-benzene; and it also comprises method of making an improved oil wherein such ortho-aminophenyl alkyl thioether is incorporated in the oil prior to application of the lubricant to a bearing; all as more fully hereinafter set forth and as claimed.

Recent developments in the design of mechanical equipment for generating and transmitting power, and particularly in the automotive field, have necessitated new bearing metals with special properties in this relation. Among these new bearing materials are binary and ternary alloys of the metals mentioned above. Cadmium-silver-copper, cadmium-nickel-copper, copper-lead-nickel, etc., alloys are in use. One ternary alloy current used in automobile engines is an alloy of cadmium with minor amounts of both silver and copper. Under the conditions imposed by modern engineering design, these new alloy bearings are commonly subjected to more severe operating conditions than were usual in the older art: to higher bearing loads, higher rubbing speeds and higher temperatures of operation. It is found that in actual use under these conditions there often develops quite serious destructive action on the bearing surface by mineral lubricating oils, even by those standard commercial oils giving particularly good results with the older bearing metals under the earlier operating conditions. The destruction of the bearing metal probably results from action of deterioration products developed in the oil. An object achieved in the present invention is the production of lubricating oils improved for these newer conditions of use and which are characterized by reduction or elimina-

tion of destructive action on the newer bearing metals by deterioration products in the oil.

We have discovered that the alkyl thioethers of ortho-amino benzene, incorporated with lubricants, are capable of achieving the objects of the present invention, the alkyl thioethers such as those containing the various amyl groups being particularly effective. By adding small amounts of such a thioether to the mineral oil or lubricant, we obtain improved lubricating compositions which satisfactorily lubricate alloy bearings. Incorporated in mineral oil, these thioethers retard destruction of the bearing metal. Also, the film strength of the lubricant is increased, the thioethers imparting extreme pressure characteristics to the oil. The character and amount of added improvement agents, here employed, are such that the normal physical properties of the oil, such as viscosity, gravity, color, etc., are not substantially altered. Certain properties of the lubricant are improved without sacrificing the other desirable properties.

We obtain improved mineral oils and lubricants suitable for lubricating such bearings under a wide range of service conditions. The new compounded lubricant satisfactorily lubricates the new alloy bearings even under high unit pressure, high bearing speeds and high operating temperatures. When prepared from suitable motor oils, the present improved compositions are excellent lubricants for the modern automobile engine. They satisfactorily lubricate the bearings without any destruction of the special bearing alloys now used, even in the presence of a free circulation of air.

Ordinarily between 0.05 and 0.50 per cent, by weight on the oil, of these thioethers is sufficient to produce a satisfactory lubricant. However, in some cases larger amounts of the thioethers may be employed, for instance, with those oils of more pronounced destructive tendency. As much as 2 per cent of thioether may sometimes be added with advantage. The particular proportions depend upon the particular thioether and lubricating base employed and the particular type of lubricant desired.

When larger amounts are employed, extreme pressure characteristics are also imparted to the mineral oil or lubricant. In many cases, the load carrying capacity of the lubricant may be in-

creased by 50 to 100 per cent. Thus the addition of the thioether gives the compounded lubricant several advantageous properties. As stated ante, even a fraction of a per cent produces the described results.

The thioethers here employed to improve the mineral oil and lubricating compositions may be represented by the following formula:

10



wherein R represents an alkyl group. As a class, these thioethers are soluble and miscible with mineral oils in substantial proportions. We have found that they are sufficiently soluble and miscible to permit incorporation with the mineral oil of an amount of thioether sufficient to obtain the described improvement.

20 These thioethers may be obtained from thioethers of ortho-nitrobenzene by reducing the nitro group to an amino group employing suitable reducing agents such as hydrochloric acid and tin, and then recovering the thioether of ortho-amino benzene so produced; the following equation illustrating the typical reaction:

30



wherein R represents an alkyl group.

In our copending application, Serial No. 98,828, filed August 31, 1936, we have described and claimed methods of preparing the said thioethers of ortho-nitrobenzene and converting them into the corresponding amino compounds and the various new thioethers so obtained.

40 In the present invention the reaction products so obtained may be employed or, if desired, they may be further purified by the various methods set forth in said application Serial No. 98,828, before incorporating them in the lubricating base.

45 As stated ante, thioethers containing alkyl groups, such as the various amyl groups, are particularly effective for the present purposes. All the amyl groups give good materials for the present purposes. Of these, the normal-amyl thioether of ortho-nitrobenzene is typical; the amyl compound has the following formula:

50



55 It is an oily liquid at normal temperatures and miscible with mineral lubricating oils. Its color is light red.

Commercial amyl preparations often contain all the possible isomers and may be used in making mixed thioethers desirable for the present purposes. There are some specific advantages both in n-amyl and iso-amyl compositions. The same is true of the thioethers derived from the butyls and propyls: each has specific advantages in certain relations. Other alkyl thioethers which are advantageous for the present purposes are

Ortho-aminophenyl-ethyl-thioether,  
Ortho-aminophenyl-butyl-thioether,  
Ortho-aminophenyl-propyl-thioether.

70 These specific thioethers, as a sub-class, may be represented by the following formula

76



wherein n is 0 to 3. However, in the broad practice of this invention other thioethers of ortho-aminobenzene may be employed.

These thioethers are quite stable, even at the elevated operating temperatures usually encountered in the lubrication of alloy bearings. Also, they are substantially neutral in reaction. Most of them are liquids at normal temperatures although some are solids melting at relatively low temperatures. Generally, their color varies from a pale yellow to a reddish yellow and when dissolved in the mineral oil, the color of the oil is only slightly altered. The amyl and ethyl thioethers are liquid; they being typical, some of their properties here important are given in the following table.

The amyl thioether is made from a commercial amyl mercaptan and contains various amyl groups.

Table A

|                           | Amylthioether | Ethylthioether |
|---------------------------|---------------|----------------|
| Gravity: °B6              | 14.8          | 24.6           |
| Viscosity, S.U.V. 100° F. | 42.8          | 39.5           |
| Pour, °F.                 | 0             | 0              |
| Color, N.P.A.             | 6             | 5.5            |
| Sulfur: Percent           | 16.4          | 20.8           |

From the above table the variation in physical properties with the length and complexity of the aliphatic constituent of the thioether is generally indicated. By employing thioethers containing other alkyl groups, these properties may be varied at will to obtain certain advantages in particular embodiments of the present invention. This may be readily done by selecting the desired mercaptan in making the thioether by the reactions described ante.

Generally, the thioethers here employed are readily miscible and compatible with petroleum oils in the percentages necessary for the present purposes. They may be incorporated with the mineral oil or lubricating base in any suitable manner. They may be dissolved in the oil by simply mixing the thioether with the oil and slightly warming with agitation to obtain uniform lubricants. Warming to temperatures between 100° F. and 180° F. is usually sufficient; the thioethers being readily soluble. With the heavier and more viscous lubricating oils this warming is advantageous since the heating lowers the viscosity of the oil facilitating the blending. In some cases, the thioethers may be dissolved in suitable volatile solvents and the solution added to the oil, the solvent being subsequently distilled off. This solvent method is particularly effective with the solid thioethers. Also, the thioethers may be first dissolved in a suitable lubricating oil to form a master batch which is subsequently blended with more lubricating oil to give a range of lubricating compositions as desired. Likewise the compounded lubricant may be converted into thickened compositions or greases in any of the usual ways. Sometimes the thioether may be directly added to metal soap greases or other compounded lubricants in which a petroleum oil is the lubricating base.

In the practice of the present invention any suitable lubricating oil base may be employed, either heavy or light oil. Ordinarily it is best to select a good grade of lubricating oil which has suitable initial properties for the particular lubrication requirement. Then the addition of the thioether produces the additional desired charac-

- teristics of restraining their destructiveness toward the newer alloy bearing metals, etc. That is, petroleum oils and lubricants of the usual grades may be employed in practicing this invention.
- 5 The oils falling within the well known S. A. E. classification are among those which can be advantageously improved by our invention. Likewise, special lubricants such as obtained by blending certain non-petroleum oils with mineral oil
- 10 may be improved by the addition of these thioethers.

The deterioration of bearings by particular oils under drastic service conditions may be readily observed by visual inspection, but a special laboratory test is necessary to readily and quickly determine it on a standard, comparable and reproducible basis and to really evaluate commercial lubricants for such alloy bearings. We have devised a satisfactory accelerated test procedure

20 which is as follows.

An alloy bearing shell of certain commonly used standard dimensions is submerged in 300 cc. of the oil or oil composition in a 400 cc. pyrex beaker and heated in a thermostatically controlled oil bath to 175° C. (374° F.) and air, at the rate of 2000 cc. per hour, is bubbled through the oil in contact with the bearing shell. At the end of 48 and 96 hours, the loss of weight and the condition of the bearing shell are determined. This

30 test will hereinafter be referred to as our standard laboratory test.

In determining the loss in weight the bearing shell is washed free of oil and dried before weighing.

When determining the effectiveness of various improvement agents the usual procedure is to run a "blank" test simultaneously with the oil composition being tested, employing for that purpose a sample of the untreated oil.

40 In such tests it is advantageous to employ commercial bearing shells. These shells comprise a suitable metal backing faced with the alloy bearing metal. In the above test, the air is bubbled against the alloy bearing face. In this way, the actual bearing face is subjected to severe deteriorative conditions. By comparison of the results of such tests with actual service tests, we have found them to be in substantial agreement as to the suitability of particular lubricants.

50 In testing our lubricants, we have employed, among others, bearings of the following approximate composition:

1. Cadmium-silver alloy. C-S 7610.

|         | Per cent |
|---------|----------|
| Cadmium | 98       |
| Silver  | 1        |
| Copper  | 1        |

60 2. Lead-copper alloy. 9020 CA.

|        | Per cent |
|--------|----------|
| Lead   | 45       |
| Copper | 53       |
| Nickel | 2        |

65 Such alloys are used in the tests of illustrative improved lubricants given post. In such tests the loss in weight, while not extremely high when expressed as "per cent loss", is nevertheless very significant, as the bearing shells used have an alloy facing of only 0.008 in. to 0.012 in. thickness on a highly resistant backing and the observed losses in the reported tests often represent a loss of the order of 10 per cent of the alloy facing.

70 75 The specific examples and tests given post are

illustrative of the detail embodiments of the present invention.

Example 1.—Into a suitable vessel there were introduced 1000 gallons (approximately 7200 lbs.) of Pennsylvania motor oil S. A. E. 10 grade and the oil was warmed to 160° F. Then 15.3 pounds of the amyl thioether of orthoaminobenzene (0.20 per cent by weight on the oil) was gradually added and the mixture agitated until a uniform blend was obtained; about one hour being required. In agitating the mixture ordinary mechanical agitators may be employed or a current of air may be passed through the warm mixture, to produce uniform blending. The amyl thioether used in this example had the properties given in Table A ante and was a mixture of isomeric amyl compounds, it being prepared from a commercial mercaptan.

The properties of the original and improved motor oil are as follows:

10

15

20

Table B

|                         | Original oil | Improved lubricant | 25 |
|-------------------------|--------------|--------------------|----|
| Gravity: °API           | 33.1         | 33.1               |    |
| Viscosity, S.U.V.:      |              |                    |    |
| 100° F.                 | 180.2        | 180.0              |    |
| 210° F.                 | 46.2         | 46.0               |    |
| Flash, O. C.: °F.       | 420          | 420                |    |
| Fire, O. C.: °F.        | 490          | 490                |    |
| Pour: °F.               | 0            | 0                  | 30 |
| Color: N.P.A.           | 1.25         | 1.50               |    |
| Carbon residue: Percent | 0.02         | 0.02               |    |
| Neutralization No.      | 0.01         | Nil                |    |
| Copper strip test       | Satisfactory | Satisfactory       |    |

From the above table, it is clear that the addition of the amyl thioether of ortho-aminobenzene does not substantially change the commonly determined physical properties of the oil. When tested by the standard laboratory test given ante, using a commercial bearing shell faced with a cadmium-silver alloy (C-S 7610), the following results were obtained in a 48-hour test run on the original oil and on the improved lubricant:

Table C

45

| Bearing shell weight—           | Original oil            | Improved lubricant |  |
|---------------------------------|-------------------------|--------------------|--|
|                                 |                         | Grams              |  |
| Before test                     | 27.5603                 | 27.3155            |  |
| After test                      | 27.0818                 | 27.3145            |  |
| Total change                    | -0.4785                 | -0.0010            |  |
| Comment                         | Substantial loss        | Insignificant loss |  |
| Bearing appearance (after test) | Badly etched and pitted | No change          |  |

55

From the above results, the beneficial effect of the thioether as an improvement agent for the oil is quite apparent. This improved lubricant when tested in an automobile engine equipped with like bearings was highly satisfactory and no destructive effect on the bearing was observed after a severe test run. Thus the standard laboratory test and actual service test gave similar results.

The improved motor oil obtained in Example 1 also has increased film strength and load carrying capacity, that is, the incorporation of the said amyl thioether imparted extreme pressure characteristics to the lubricant. This is one of the advantages of employing these thioethers of ortho-aminobenzene.

Example 2.—Employing the same blending procedure as for Example 1 and substituting a highly refined motor oil of S. A. E. 30 grade made from Pennsylvania crude and incorporating 1 per cent

60

65

70

75

of amyl thioether of ortho-aminobenzene, we obtain an improved lubricant having marked extreme pressure characteristics.

When tested in the Almen lubricating testing machine using the Almen technique (a standard test), the increased load carrying capacity over that of the original oil is apparent. In this test the original oil withstood a load of only 8 pounds whereas the improved lubricant withstood a load of 16 pounds under similar conditions. These weight loadings on the Almen lubricating testing machine produced bearing loads respectively of 4000 pounds per square inch and 8000 pounds per square inch. Clearly, very small proportions of these thioethers of ortho-aminophenyl alkyl thioethers are capable of improving the film strength and load carrying capacity of highly refined lubricating oils by 50 to 100 per cent.

*Example 3.*—Employing the procedure of Example 1 and substituting a highly refined Pennsylvania motor oil S. A. E. 20 grade in lieu of the lubricating base employed in Example 1, still another improved lubricant is obtained.

In the above examples, other thioethers may be used in lieu of the amyl derivative and similar improvements obtained.

The above examples are but illustrative embodiments of the present invention and in practice other embodiments may be used. That is, the percentage of thioethers employed may be varied as indicated, according to the particular properties desired in the final lubricant. Likewise, the lubricating base itself may be selected according to the type of final lubricant to be produced. For instance, any of the usual greases or the usual blends of mineral and non-mineral oils may be employed as a lubricating base in making lubricants of our improved type. The addition of the thioethers to these lubricating bases produces a like improvement in film strength and reduces their destructiveness toward the newer bearing alloys. When incorporating the thioethers in a grease composition or like thickened lubricant, mechanical agitators rather than a current of air are employed to obtain uniform mixing and blending. That is, the thioether and grease may be compounded in the usual mixers such as blade mixers, equipped with heating jackets. However, in making such greases the thioethers may advantageously first be incorporated with the oil base according to the procedure of Example 1 and then the metal soap or the thickening agents added to the improved oil, in the ordinary way to produce the desired grease compositions. In other words, the improved mineral oils of the present invention may be used in lieu of the ordinary oils in making special lubricating compositions such as greases, etc.

60 The ethyl thioethers of orthonitrobenzene and other thioethers may be employed in lieu of the amyl thioether in the examples given ante. The amyl and like alkyl thioethers being particularly effective are ordinarily employed. With proper blending, good lubricants may be produced with all these thioethers compounded with various petroleum oils or mineral oil lubricants.

As stated ante, the incorporation of these thioethers with the lubricating base produces several improvements in the final lubricant without deleteriously affecting the desirable properties. While the exact reasons for the improvements obtained are not fully known, we are satisfied with observing and utilizing the actual improvements ob-

tained by adding and incorporating these thioethers with commercial lubricants.

The improved performance of lubricants secured in the presence of the newer alloy bearing metals by means of our present invention appears to result from the presence of an aryl thioether having a second substituent group in the ortho position to the said thioether group. In the present invention we claim specifically the use of materials wherein the substituent group ortho to the thioether group is an amino group. In our copending application Serial No. 98,826, filed August 31, 1936, we describe and specifically claim materials wherein the substituent group is a nitro group. Certain special advantages are secured with each of these types of materials.

Having described the methods of making and using such improved lubricants, what we claim is:

1. A method of lubricating bearing surfaces in internal combustion engines when subjected to conditions of operation which comprises maintaining between bearing surfaces, one of which is an alloy formed chiefly of a metal of the class consisting of cadmium and copper, a film of a lubricating oil which initially produces an effective lubricating action but which would normally tend to corrode the aforesaid alloy, and maintaining the effectiveness of the lubricating oil by means of between .02 per cent and 0.20 per cent, by weight on the oil, of an ortho-aminophenyl alkyl thioether dissolved in such lubricating oil, said alkyl thioether having the following formula:



35

wherein R represents an alkyl group.

2. A method of lubricating bearing surfaces in internal combustion engines when subjected to conditions of operation which comprises maintaining between bearing surfaces, one of which is an alloy formed chiefly of a metal selected from the class consisting of cadmium and copper, a film of lubricating oil which initially produces an effective lubricating action but which would normally tend to corrode the aforesaid alloy and maintaining the effectiveness of the lubricating oil by incorporating therein ortho-amino-phenyl amyl thioether in a small but sufficient proportion substantially to retard the corrosion.

3. As a new and improved lubricant capable of lubricating cadmium-silver and other special alloy bearings at high temperatures, pressures and speeds, without corroding such alloy bearings, an improved motor oil comprising a mineral oil containing a minor amount of an alkyl thioether of ortho-amino benzene dissolved therein, said mineral oil being a motor oil which while capable of initially producing an effective lubricating action, would normally tend to corrode said alloys, under said conditions, and the amount of said thioether being sufficient to effectively and substantially retard the destructive action on said alloy bearings which would normally occur in the absence of said thioether, said alkyl thioether having the following formula:



70

wherein R is an alkyl group.

4. As an article of manufacture, a new and improved lubricant comprising a major propor-

tion of a mineral lubricating oil containing a minor proportion of an ortho-aminophenyl alkyl thioether dissolved therein, said thioether having the following formula:

5



wherein R represents an alkyl group, and the amount of said thioether being sufficient to substantially improve the lubricating qualities of said lubricating oil.

5. The new and improved lubricant of claim 4 wherein said mineral lubricating oil contains from 0.02 to 2 per cent of said alkyl thioether of ortho-aminobenzene dissolved therein.

6. The new and improved lubricant of claim 4 wherein said thioether is ortho-aminophenyl amyl thioether.

7. The new and improved lubricant of claim 4 wherein said thioether is ortho-aminophenyl ethyl thioether.

TROY LEE CANTRELL.  
JAMES OTHO TURNER.

10

5